

## UNITED STATES PATENT OFFICE

2,179,314

## PROGRESSIVE-BURNING SMOKELESS POWDER

Elton R. Allison, Kenvil, N. J., assignor to Hercules Powder Company, Wilmington, Del., a corporation of Delaware

No Drawing. Application October 6, 1938,  
Serial No. 233,597

3 Claims. (Cl. 52—5)

This invention relates to smokeless powder, and particularly to coated, deterred, or progressive-burning smokeless powder.

Smokeless powder, on combustion in the chamber of the gun in which it is used, tends to burn initially at a more rapid rate than is desired and thus produces high breech pressures. This defect is not overcome by using larger grains of powder, in the case of those powders intended to give maximum results in center-fire rifle cartridges. Many attempts have been made in the past to deter the initial rate of burning of the powder grains by coating said grains with an agent, explosive or non-explosive, which will slow down the initial rate of combustion of the powder grains, thus extending the period of time taken by the grains to burn completely, and in this way reduce the otherwise high breech pressure in the gun. The coating material used penetrates the powder grains more or less, so that, as the powder grains burn, the successively exposed surfaces contain gradually, less and less of the deterrent material, thus causing subsequent combustion of the powder grain to proceed with increasing speed as the bullet travels down the bore of the gun.

In the past, many substances have been used, without complete success, to coat smokeless powder grains, e. g., such materials as diethyldiphenylurea, dimethylidiphenylurea, dinitrotoluene, alkyl phthalates, or mixtures thereof, and various methods of applying such deterrent substances have been known.

The known methods of deterring or coating smokeless powders have not been completely effective in that they have not produced smokeless powders of high gravimetric density combined with high ballistic stability. By ballistic stability is meant the maintenance, with age, of the initial ballistics produced by the powder. For example, many of the coating agents continue to penetrate into the powder grain, particularly in warm climates, and thus alter their deterrent characteristics.

With modern loads of deterred smokeless powder it is usual to find that the maximum velocity which can be obtained with a given projectile is limited, not by the maximum allowable pressure produced in the chamber of the gun, but by the powder capacity of the cartridge. However, an increase in the gravimetric density of the powder would permit the use of greater powder charges and result in an increased velocity of projectile.

It is the object of this invention to produce

a coated smokeless powder which is ballistically stable with age and of high gravimetric (or loading) density. The high gravimetric density of my coated powders enables me to use greater charges than hitherto permitted by the volumetric capacity of the cartridge, which is a distinct improvement over prior art powders and an advantage which has been sought for many years by the art. My improved smokeless powder is not subject to clustering or sticking together of the grains. 5

In the preparation of coated smokeless powder in accordance with my invention I use coumarin as the coating agent. This compound may be used alone or in combination with other coating 15 agents.

I may use as the powder grains to be coated either a single base (nitrocellulose) powder or a double base (nitrocellulose-nitroglycerine) powder. Although the powder grain may be of 20 any size I have found that my coating agent offers the most advantage when used with the larger caliber powders.

In practicing my invention, coumarin is applied to the smokeless powder as a solution thereof in a volatile solvent which is substantially a non-solvent for the smokeless powder. Among the volatile solvents which I have used are toluene, ethylene dichloride, petroleum naphtha, isopropyl alcohol, water, and ethyl alcohol, and 30 of these I prefer using 95% by volume ethyl alcohol.

To 100 parts by weight of smokeless powder I add from about 1 to about 10 parts by weight of coumarin dissolved in a suitable quantity of solvent. The smokeless powder is treated with coumarin in any suitable manner, for example by tumbling the powder and the coumarin solution in a barrel at a temperature within the range of from about 10° C. to about 95° C. for a period 40 of time between about 5 minutes to about 4 hours, after which the powder so coated may be subjected to further heat treatment to eliminate any remaining solvent, if this appears desirable. The time and temperature of treatment as well as the 45 quantity of coating will necessarily be varied with the size of the powder grain employed, the type of firearm in which the powder is to be used, etc. In the case of application of extremely heavy 50 coatings to the powder, when using a volatile solvent other than water, water may be added to the coated powder grains before elimination of the volatile solvent in order to prevent sticking and clustering of the grains. 55

As specific illustrations of the carrying out of my invention, the following examples are given:

*Example 1*

Nine hundred and seven parts by weight of a double base smokeless powder containing 20% nitroglycerine pressed through a 0.045 inch die having a 0.015 inch pin, and the strand so produced cut into 11 particles per inch was placed in a sweetie barrel maintained at 75° C. and to this was added 45.3 parts of coumarin dissolved in 160 parts by weight of ethyl alcohol, the mixture tumbled in the closed sweetie barrel for about 1/2 hour at 75° C. then for another 1/2 hour at 90° C., after which time the powder was removed to a dry house and dried for 3 days at 55° C., then graphited, screened, and exposed to an atmosphere of 50 to 60% relative humidity to bring the moisture content to equilibrium. A yield of 95% of unclustered powder was obtained having a gravimetric density of 0.944.

*Example 2*

As a comparison with the above example I coated 907 parts by weight of the same smokeless powder as above in the same manner indicated before with 45.3 parts by weight of symmetrical diethyldiphenylurea (Centralite #1). A yield of 38% of unclustered powder was obtained having a low and unsatisfactory gravimetric density of 0.919.

The powders prepared in accordance with the two examples above were fired in a .30 caliber—1906 cartridge case using a 110 grain bullet, the cartridge being loaded in each case with sufficient powder to fill said cartridge to the base of the bullet. The results obtained are shown in the following table:

| Powder from—   | Charge in grains | Mean velocity over 153 foot range | Mean pressure        |
|----------------|------------------|-----------------------------------|----------------------|
| Example 1..... | 62.5             | Ft./sec. 3,435                    | Lbs./sq. inch 50,800 |
| Example 2..... | 61.1             | 2,880                             | 26,900               |

It will be noted in the above table that a powder coated with coumarin as disclosed by the present invention has an appreciable velocity increase over comparator Example 2 in which a prior art coating material is used. Furthermore, in comparison with Example 2 it will be noted that a greater charge of powder can be utilized in the same space in the cartridge in the case of Example 1, which is, of course, due to the higher gravimetric density of the powder prepared in accordance with this invention.

To illustrate the improvement in stability obtained by my coated powder, I subjected it to warm storage using for comparison a powder coated in the same manner with butylphthalyl butylglycolate. The results of this test are shown in the following table:

| Coating agent                     | Days storage at 50° C. | Pounds per square inch pressure increase | 20 |
|-----------------------------------|------------------------|------------------------------------------|----|
| Coumarin.....                     | 62                     | 100                                      |    |
| Butylphthalyl butylglycolate..... | 62                     | 7,600                                    | 25 |
| Do.....                           | 90                     | 8,900                                    |    |

The marked improvement in ballistic stability is apparent from the above table. It will be understood that the foregoing are by way of illustration only and that the scope of my invention is not to be limited thereto, except as hereinafter defined by the claims.

What I claim and desire to protect by Letters Patent is:

1. Smokeless powder grains surface coated with coumarin.
2. Double base smokeless powder grains surface coated with coumarin.
3. Smokeless powder grains surface coated with coumarin in amount from about 1% to about 10% by weight of the powder.

ELTON R. ALLISON. 45